

## UNITED STATES PATENT OFFICE.

LEON CAMMEN, OF NEW YORK, N. Y., ASSIGNOR TO THE INTERNATIONAL NICKEL COMPANY, A CORPORATION OF NEW JERSEY.

## NICKEL ALLOY.

No Drawing.

Application filed February 7, 1921. Serial No. 443,251.

*To all whom it may concern:*

Be it known that I, LEON CAMMEN, a citizen of the United States, and resident of borough of Manhattan, in the city, county, and State of New York, have invented certain new and useful Improvements in Nickel Alloys, of which the following is a specification.

This invention refers particularly to ternary alloys of nickel, copper and aluminum, wherein the aluminum is present not merely as a residue of the process of deoxidation, but a necessary constituent of the alloy.

The use of aluminum in very small amounts, usually under one per cent, in copper-nickel alloys, is not new, it being introduced just previous to casting as a purifier and deoxidizer. When aluminum is so used, the effort is however made to introduce as little of it as possible, the ideal being to put in just enough Al to take out all the oxygen present in the metal bath. One per cent is now considered in Monel metal foundries to be about the limit of the amounts in which either aluminum or magnesium should be used as deoxidizers (all percentages are by weight).

In the present specification is however described an alloy containing from 3 to 17 per cent of aluminum in addition to nickel and copper.

As a base for the production of such alloys is used Monel metal which is a trade name of an alloy containing 25 to 28 per cent of copper, 65 to 69 per cent of nickel, and some impurities, such as iron, manganese, carbon, etc. The advantage of using this particular alloy in the production of nickel-copper-aluminum alloys lies in the fact that the percentages of nickel and copper in the monel are satisfactory for purposes of producing the ternary alloy, and that Monel metal is cheaper than would have been an alloy of similar composition made from copper and nickel. As far as the properties of the ternary alloys are concerned, however, it does not make any difference whether the alloy is made with such a natural alloy of copper and nickel as Monel metal, or from synthetic alloys of the two metals.

The preferred content of nickel in the final alloy is from about 60% to about 70%

and that of aluminum is from about 10% to 3%.

In my tests I have found that the addition of aluminum to copper-nickel alloys of the composition approaching that of Monel metal, which hereafter (including the claims) will be designated as Monel metal, begins to affect the properties of the alloys when the content of aluminum is in excess of 3 per cent, the metal becoming harder and denser in structure. Finally at about a content of 8 to 10 per cent of aluminum, the metal becomes so hard that it cannot be cut with a hacksaw or filed, and if an attempt to file it is made, it turns the teeth of the file. On the other hand, however, the metal, while so hard, is tough and extremely resistant to shock, which makes it of value in construction. It also retains the ability of standard Monel metal to resist corrosion.

As regards the methods of production of the metal, I have found that the simplest way is to add the proper amount of aluminum, molten, to a molten bath of Monel metal, carefully stirring the mixture. A powerful reaction rapidly sets in, the surface of the pot of mixture becoming of a brilliant white color, after which there is often a tendency for the mixture to freeze. The copper-nickel-aluminum alloy casts well, and has no special tendency towards the formation of blow-holes.

My tests have shown that an addition of aluminum in percentages in excess of 17 per cent produces a brittle alloy.

I claim:

1. An alloy of nickel, copper and aluminum, wherein the content of nickel is in excess of 50% and the content of aluminum is not less than about 3% and not more than 17%, the predominant metal of the remaining content being copper.

2. An alloy of nickel, copper and aluminum, wherein the content of nickel is not less than 55%, the content of copper is not less than 18% and the content of aluminum is not less than about 3%, the three metals named forming the predominant percentages of the alloy.

3. An alloy of nickel, copper and aluminum, wherein the content of nickel is not substantially less than 50% and the con-

tent of aluminum is about 4% to 5%, the predominant metal of the remaining content being copper.

4. An alloy of nickel, copper and aluminum, wherein the content of nickel is 60% to 70% and the content of aluminum is 10% to 3%, the predominant metal of the remaining content being copper.

5. An alloy of nickel, copper and aluminum, wherein the content of nickel is in excess of 50% and the content of aluminum is not less than about 3% but is insufficient

to destroy the malleability of the alloy for mechanical working, the predominant metal of the remaining content being copper.

15

Signed in New York, in the county and State of New York, this 5th day of February, A. D. 1921.

LEON CAMMEN.

Witnesses:

ERNEST HARTFORD,  
A. L. SCHUMACHER.